

## UNITED STATES PATENT OFFICE.

JULES ERNEST HESSE AND MATHIAS PARAF-JAVAL, OF PARIS, FRANCE,  
ASSIGNORS TO JEAN DIEDERICHS, OF LYONS, FRANCE.

## PROCESS OF TRANSFERRING AND PRINTING.

SPECIFICATION forming part of Letters Patent No. 748,604, dated January 5, 1904.

Application filed September 16, 1899. Serial No. 730,764. (No specimens.)

*To all whom it may concern:*

Be it known that we, JULES ERNEST HESSE and MATHIAS PARAF-JAVAL, of the city of Paris, in the Republic of France, have invented a new and useful Improvement in Processes of Transferring and Printing, which is fully set forth in the following specification.

The present invention has relation to the use for printing and transfer of ordinary dyeing colors with a view to obtaining a greatly improved final product.

All inks used in lithography are insoluble and incapable of dyeing (in its proper sense) textile fabrics, because their adhesion thereto is due only to the varnish. Such products are not capable of withstanding the usual cleansing operations and agents as rubbing and soaping or the action of hydrocarbons or carbon sulfid or bisulfid or the like, because these agents effect the separation of the coloring-matter and varnish from the fabric. Further, in these cases where the inks are fixed to the fabric by the adhesion of the varnish thereto the fabric is not only stiffened by the varnish, but the beauty and purity of the colors are reduced. The lithographically-printed products, on the other hand, are of a degree of fineness and softness which cannot be attained by any other process of printing.

In the usual fabric-printing establishments the coloring-matter dyes (in its proper sense) the fabrics in that the dyestuff does not adhere thereto mechanically only, as in lithographic printing. The thickening generally employed disappears during the usual final processes (washing, soaping, lustering, &c.) which are resorted to for the elimination of the thickening. Of the image there remains, therefore, only the combined colors upon the printed surface. In this case it seldom occurs that the coloring does not actually dye the fabric and that such coloring-matter adheres to the fabric through the thickening, as so-called "plastic" colors—cinnabar, ultramarine, and lampblack, thickened with albumen, casein, gluten, &c.—are used.

From what has been said it will be seen that in the usual method of printing on fabrics there is neither stiffness nor impurity nor

non-transparency nor cloudiness, yet the prints lack the fineness and softness obtainable by the lithographic process; and it is the object of our invention to obtain a product which while having the fineness and softness of the lithographic products and which will be actually dyed, as in the usual printing methods, at the same time will be free from the undesirable features of the two processes.

Attempts have been made, but without success, to substitute for the insoluble lithographic inks the tannic-acid salts of the basic artificial dyes of the type of tannic-acid rosanilin and mauvein. This class of dye-stuffs is a very large one, yet readily recognizable if their aqueous solutions are reacted upon with a tannic-acid solution, and if a precipitate difficult of solution when cold is obtained it is conclusive proof that it is one of those which can be used in carrying out the present invention. Though these tannates are only slightly soluble when cold, they are sufficiently soluble when warm, and we avail ourselves of this characteristic in the carrying out of our process. Instead of using these basic colors in the form of tannates we convert the same into other lakes which are capable of readily yielding up their coloring-matter. We have also found that in this manner we are enabled to make use of all coloring-matters, even the non-basic. The base of this lake is an indifferent body, as pipe-clay, porcelain-clay, carbon, &c., colored in a solution of any desired coloring-matter which can best be effected while hot, and during the cooling the material is stirred. The lake is then washed in cold water and filtered, pressed, and dried and mixed with lithographic varnish by rubbing, as usual. The function of the varnish is to temporarily retain on the paper from which the color is to be transferred to the fabric to be dyed the soluble colors employed. The base of the lake, pipe-clay, &c., which but feebly retains the soluble coloring-matter, is mixed with the varnish, and consequently adheres to the paper with it. The only matter transferred to the fabric from the transfer-paper is the soluble part of the color which is retained by the base of the lake. The varnish and the base adhere to the

paper. We obtain the same results with substances of animal origin, as albumen, glue, casein, the solutions of which we color with the dissolved dyestuffs, then allow it to dry 5 and mix it with varnish.

The following will serve as a description of animal-black lake: Rosanilin or its salts may serve as an example, though, as will be readily understood, any other coloring-matter may be used. The proportions of carbon and coloring-matter may vary within very wide limits without affecting the result. One hundred grams rosanilin hydrochlorate are dissolved in from ten to fifteen liters of 15 boiling water, and to this is added from six hundred to eight hundred grams animal-black previously purified by means of hydrochloric acid. The mixture is kept at the boiling-point for fifteen minutes, stirred, and then 20 allowed to cool, while being constantly stirred. After settling, the liquid is decanted, and this will be but slightly colored if the black is of good quality. The carbon precipitate is at once filtered, pressed, and dried. 25 The quantity of varnish employed in the fabrication of the lake varies. In the case of rosanilin, for example, the quantity varies according to the depth of shade desired, according to the thickness of the fabric, and 30 according to the degree the design is to be brought out or developed. For a red, a little more intense than medium, one or two parts of the lake or tannate of rosanilin are mixed with eight or nine parts of lithographic varnish. If it is desired to obtain a paler 35 red or even a rose, more or less varnish would be added to the mixture. In any event the proportions must be practically determined in each case, since they vary with 40 the intensity and duration of the pressure, the temperature, and the degree of impregnation of the fabric with the transfer liquid hereinafter referred to.

The majority of colors, also the natural 45 colors—as indigo, carmine, &c.—yield lakes which are particularly adapted to the carrying out of this invention. All these carbon lakes, although faultless for fabrics of animal origin—as silk, for example—do not combine 50 with vegetable fiber. This disadvantage we have remedied in that we treat the fabrics of vegetable origin first with tannate of tin or antimony. To this end we treat vegetable fabrics in the manner above described with the aid of sodium stannate (stannate of soda) and 55 sulfuric acid. After drying we block the fabric twice without washing or drying in a solution of one hundred grams of tannin in ten liters of water, which operation is repeated twice at an interval of half an hour. 60 After the lapse of another half-hour the fabric is washed and drawn in an unfolded state through a bath composed of from one and one-half to two and one-half parts tartar emetic in one hundred liters of water. This 65 drawing of the fabric through the bath is ef-

fected at a sufficiently slow rate that each part of such fabric will remain a quarter of an hour in the bath, after which the fabric is washed and dried.

All carbon lakes capable of combining with tin or tannic acid can be used for printing upon fabrics treated with tin or antimony tannate, and the colors are found in the fabric in the same condition as when printed in 75 the usual manner.

Where we use the animalizing process with vegetable-fiber fabrics usually employed for printing upon, we attain the same good results. This animalizing process is carried 80 out by blocking the fabric in a solution of one part albumen in ten parts water. The albumen is then allowed to set. The carbon colors yield their coloring-matter to the albumen, which adheres very firmly to the fabric; but 85 these transfers lack the genuineness of the metallic tannic-acid salts.

Whatever may be the nature of the mordant or the composition of the transfer-lake, we found that the feeble gumming which printers give to their materials and which does not take up water readily also facilitates our lithographic transfer.

For the purpose of gumming we repeatedly pad the fabric without intermediate drying 95 in a solution of from five to twenty-five grams gum-tragacanth in one liter of water. The stuff is carried each time under a roller at the bottom of the bath and then squeezed out between two padding-cylinders, after which the 100 stuff is dried in a drying-cylinder. The object of this gumming is well known. The small air-bubbles on the surface of the fabric are driven off and replaced by a fine layer of gum-tragacanth.

Any other gum can replace the gum-tragacanth, and the effect can be heightened by addition to the gum solution of a substance which facilitates the solution of the color to be printed—as, for instance, glycerin in the 110 proportion of from five to twenty-five grams per liter. The gumming also facilitates the taking up of the liquid with which the fabric is moistened before being printed upon. This liquid, which supplies the means necessary to the solution and diffusion of the colors, may be composed as follows: seven hundred grams acetic acid; three hundred grams alcohol, 75° Baumé; five to twenty grams gum-tragacanth, and fifteen grams glycerin 115 or glycol. The gum is first swelled in some water and is then slowly added, under constant stirring, to the glycerin, acetic acid, and finally diluted with water. If the action of this liquid is to be increased, the proportion of one or the other of the acid salts mentioned is added in small quantities. Just before printing we impregnate the fabric with the liquid, and this impregnation should be uniform and can readily be effected by hand-pressure and with a printing-block lined with 120 125 130 135 felt.

The printing is facilitated when the paper from which the color is to be transferred to the fabric to be dyed is moistened about half an hour before transferring by spraying on the back thereof a transfer liquid free from gum. This liquid, which may also consist of an aqueous solution of from two per cent. to twelve per cent. of acetic acid, facilitates the removal of the soluble color from the paper in printing.

In the printing of fabrics by means of cylinders or rollers the pressure-cylinder, of metal, presses the fabric to be printed almost directly into the deeply-graven printing-cylinder through a cloth blanket and a runner, and the finer and deeper the engraving the tighter and thinner the clothing. Accordingly we provide the lower plate of the press with a lead plate having accurately-parallel surfaces which has not only for its objects the correct positioning thereon of paper and fabrics, but also acts as an intermediate piece which enhances the action of the pressure-blanket and runner. Upon this lead plate are laid from two to five sheets of writing-paper and upon the latter two or three sheets of fine calico. Upon the bed so formed is placed the fabric to be printed and previously impregnated, as above set forth, and upon this is placed the lithographic print. On the back of the latter are placed two or three sheets of calico and a few sheets of writing-paper, and upon the whole is placed a lead plate similar to the one on the bed-plate of the press, and then follows the actual transfer.

Inasmuch as the greatest pressures produce only bad results and it is necessary to allow the fabric to absorb the coloring constituents, we adopt a means also resorted to in dyeing and calico-printing in order to facilitate this actual dyeing. Heat is applied in the form of boiling water or in the form of steam, and to this end both metal plates of the press are so arranged as to be heated by a steam-heater coil, for which of course any other system of heating can be substituted.

The water and other liquids used for impregnating the fabric diffuse more readily through the printing-varnish and the base of the lake and dissolve more coloring-matter when heated than when cold. The fabric while being dyed takes up the coloring-matter from the solution until finally all the coloring-matter on the transfer-paper is absorbed and until the fabric is saturated with coloring-matter. Hence an actual dyeing of the fabric takes place. The hot vapors of the transfer liquid effect the steaming of the fabric, as is done in calico-printing.

We have found that by hot printing the actual pressure is materially reduced, and this renders the repeated use of the transfer-paper possible.

It frequently happens that the transferred colors dye the fabric but partially, and to avoid this we treat the pressed and dried fab-

ric in a well-known manner, as if it had been printed with steam-colors—namely, the fabric is hung in a moist chamber heated to form about 25° to 50° centigrade and allowed to remain therein until the dyeing is as uniform as possible—or the fabric may be steamed, as is done in fabric-printing. If this be the case, which can be determined by subjecting a piece to the cleaning process, the fabric is finally subjected to said latter process.

If the colors used are tannic-acid colors and if the fabric has not previously been mordanted with tin or antimony, the tannic-acid colors are fixed upon the fabric by drawing the same through a solution of tartar emetic, after which the fabric is washed. When, however, tannic-acid colors are printed upon fabrics mordanted with tin or antimony, they are washed without passing them through the fixing solution of tartar emetic. This washing is effected in a large quantity of water in order that the base or ground of the fabric which did not receive the transfer may not be colored.

For the purpose of fixing or clarifying we use a twenty-five per cent. to one-hundred per cent. bran-water, which is renewed whenever it begins to color, or, instead of the bran liquor, pure or distilled water can be used containing from one to two parts of soap to one hundred parts of water. The fabric is then washed at a temperature of from about 30° to 60° centigrade and the soap-water is renewed as soon as it ceases to foam strongly or as soon as it begins to color. The fabric is then washed and dried. If for any reason a small amount of the lithographic varnish should be transferred to the fabric with the soluble colors, this washing readily removes it.

Should the fabric from any cause show spots which may be produced by the action of the tannic acid upon iron, said fabric is drawn through a solution of tin chlorid (two grams tin chlorid per liter of water) until the spots disappear, after which the fabric is washed.

If paper is used instead of a fabric in the described transfer process, faultless imitations of water-color paintings are obtained.

What we claim is—

1. The process of producing designs or patterns on fabrics, consisting in first forming a print upon a suitable material with a lake of the desired coloring-matter capable of yielding up its coloring-matter, and then transferring the design or pattern to the fabric.

2. The process of producing designs or patterns on fabrics, consisting in forming a print upon a suitable material with a lake consisting of a suitable substance colored with a suitable coloring-matter and mixed with lithographic varnish, and then transferring the design or pattern to the fabric.

3. The process of producing designs or patterns on fabrics consisting in gumming the fabric, forming a print upon a suitable material with a lake of the desired coloring-mat-

ter capable of yielding up its coloring-matter, and then transferring the design or pattern to the fabric.

4. The process of producing designs or patterns on fabrics consisting in gumming the fabric with a solution of gum to which has been added a substance capable of facilitating the solution of color to be printed, forming a print upon a suitable material with a lake 10 of the desired coloring-matter capable of yielding up its coloring-matter, and then transferring the design or pattern to the fabric.

5. The process of producing designs or patterns on fabrics, consisting in treating the 15 fabric with a suitable mordant and gumming the fabric with a solution of gum to which has been added a substance capable of facilitating the solution of color to be printed, forming a print upon a suitable material with 20 a lake of the desired coloring-matter capable of yielding up its coloring-matter, and then transferring the design or pattern to the fabric.

6. The process of producing designs or patterns on fabrics, consisting in treating the 25 fabric with a suitable mordant, forming a print upon a suitable material with a lake of the desired coloring-matter capable of yielding up its coloring-matter, and then transferring the design or pattern to the fabric.

7. The process of producing designs or patterns on fabrics, consisting in treating the fabric with a suitable mordant, forming a print upon a suitable material with a lake of 30 35 a tannic-acid color and then transferring the design or pattern to the fabric.

8. The process of producing designs or patterns on fabrics, consisting in treating the fabric with tannate of a suitable metal, forming a print upon a suitable material with a lake of the desired coloring-matter capable 40

of yielding up its coloring-matter, and then transferring the design or pattern to the fabric.

9. The process of producing designs or patterns on fabrics of vegetable origin, consisting in treating the fabric with a substance capable of causing the lake subsequently used to combine therewith, forming a print upon a suitable material with a lake of the desired 50 coloring-matter capable of yielding up its coloring-matter, and then transferring the design or pattern to the fabric.

10. The process of producing designs or patterns on fabrics, consisting in gumming the 55 fabric by passing the same through a gum solution and then squeezing it, impregnating the gummed fabric with a suitable transfer liquid, forming a print upon a suitable material with a lake of the desired coloring-matter 60 capable of readily yielding up its coloring-matter, and then transferring the design to the fabric.

11. The process of producing designs or patterns on fabrics, consisting in gumming the 65 fabric, impregnating the gummed fabric with a suitable transfer liquid, forming a print upon a suitable material with a lake of the desired coloring-matter capable of readily yielding up its coloring-matter, bringing the 70 surface of the print into contact with the fabric and transferring the design to the fabric by the application of heat and pressure.

In testimony whereof we have signed this specification in the presence of two subscribing witnesses. 75

JULES ERNEST HESSE.  
MATHIAS PARAF-JAVAL.

Witnesses:

LOUIS DOMINIQUE AUGUSTE CASALONQE,  
ANTONIO FERNANDO DE LA CALLE.